

June 30, 1931.

W. S. NUTTER

1,812,640

PILE FABRIC AND METHOD OF MAKING THE SAME

Original Filed Feb. 4 1928



Inventor.  
William S. Nutter  
by *Heard Smith & Tennant.*  
Atlys.

## UNITED STATES PATENT OFFICE

WILLIAM S. NUTTER, OF SANFORD, MAINE, ASSIGNOR TO GOODALL WORSTED COMPANY,  
OF SANFORD, MAINE, A CORPORATION OF MAINE

## PILE FABRIC AND METHOD OF MAKING THE SAME

Application filed February 4, 1928, Serial No. 252,029. Renewed January 12, 1931.

This invention relates to fabrics and especially to pile fabrics of the plush variety although it is equally applicable to other kinds of pile fabrics. A pile fabric presents a plurality of pile ends which are interlocked with interwoven filling and binder warp threads.

The color of the surface of the pile face of the fabric is determined by the color of the pile ends while the color of the back face of the fabric is determined by the color of all three threads, i. e., the pile threads, the binder warp threads and the weft threads. In order to give the back face of a plush fabric a color which harmonizes with the color of the front or pile face it has heretofore been customary to use warp threads which are dyed to the proper color. It is a well-known fact that the process of dying threads reduces their strength by approximately 25% so that dyed warp threads are more apt to break and require more careful handling in the various weaving operations than undyed warp threads. The undyed threads are, however, relatively light colored or white in appearance and consequently in a plush fabric having undyed warp threads the portions of the undyed threads which are exposed on the back face of the fabric will give a light color or tone to the back face of the fabric which may not harmonize properly with the color of the front face of the fabric that is determined by the color of the pile threads.

It is one of the objects of my present invention to provide a novel plush fabric in which light-colored warp threads such as undyed warp threads may be used but which will have a back face of a color to harmonize with the color of the pile threads, and also to provide a novel method of making such a pile fabric.

In weaving any pile fabric especially if the fabric is one in which the pile ends are formed of mohair, it has been thought necessary to use a relatively large number of binder warp threads to effectively bind the pile ends into the fabric.

Another object of my invention is to provide improvements in pile fabrics by which

the pile ends will be firmly held in the fabric with a fewer number of binder warp threads than have heretofore been thought possible.

A still further object of the invention is to provide an improved mohair pile fabric using mohair pile threads having kemp fibre therein and which is so constructed that the presence of the kemp fibres is not noticeable.

In carrying out my invention I weave the pile fabric as usual by interlocking pile ends with interwoven filling and binder warp threads, except that the warp threads are of a light color such as would result by using warp threads formed partially or wholly of undyed fibres. After the fabric has been woven I apply to the back face thereof a non-penetrative, water-resistant coating which is flexible and is not affected by heat and which also has sufficient color to color the back of the fabric to the desired shade.

While various materials having these characteristics may be used for coating the back of the fabric I will refer by way of example to a pyroxylin or nitro-cellulose composition. Such a composition makes a coating which when applied to the fabric will lie on the face thereof and will not penetrate into the fabric to any appreciable extent; it is flexible so that it will not crack by bending or folding the fabric; it is water resistant and is not affected by heat; and it also has a binding effect. Merely for the sake of convenience I will refer hereinafter to this coating material as "pyroxylin" but I wish it understood that this expression is used merely in a descriptive sense and not with the idea of limiting the practice of the invention to any particular substance.

Before the fabric has the coating applied to the back thereof the undyed or partially undyed warp threads, which are of a light or white color because of their undyed condition, show through on the back of the fabric somewhat giving it a speckled appearance which is not considered desirable and which unless corrected would render the fabric more or less unsalable.

The application of the pyroxylin to the back of the fabric provides a pyroxylin coating which is localized on the back of the

fabric since the pyroxylin does not penetrate into the fabric to any extent but in effect forms a coating on the back face only of the fabric. This pyroxylin coating 5 serves two purposes. In the first place, the layer of colored pyroxylin overlies the portions of the light-colored warp threads exposed on the back of the fabric and by so doing colors said portions so that the back 10 of the fabric presents a color which is determined by the color of the pyroxylin coating. This color, of course, can be such as to harmonize entirely with the color of the front or pile face of the fabric as determined 15 by the pile threads.

In the second place, the layer or coating of pyroxylin by its engagement with and adhesion to the portions of the warp threads, weft threads and pile threads which are exposed 20 on the back of the fabric serves to assist in tying in the pile ends and thus preventing them from becoming loosened. In fact, this tying-in effect of the pyroxylin coating is such that it is possible to produce 25 a satisfactory pile fabric by using fewer binder warp threads than has heretofore been thought necessary. In other words it is possible to initially weave the pile fabric with what would be a deficiency of warp 30 threads under normal conditions, such deficiency being made good by the binding effect of the pyroxylin.

In weaving plush fabrics it is usual to use two binder warps and a pile warp but 35 by providing the pile fabric with a coating of pyroxylin or other binding material on the back face I find that it is possible to weave a satisfactory plush fabric by using only one binder warp. The binding action 40 of the pyroxylin coating on the pile ends is sufficient so that it takes the place of the threads of one of the binder warps. The reduction in the number of warp threads obviously decreases the expense of manufacturing 45 the fabric and as the expense of applying the coating of pyroxylin or other binding material to the back of the fabric is less than the expense involved in the warp threads which may be discarded the result 50 is that with my invention it is possible to produce a satisfactory plush fabric at a reduced expense.

In the making of some pluses and other pile fabrics the pile threads are made of 55 mohair yarn, which is yarn made from the wool of the Angora goat. The Angora fleece includes not only the fine and soft hairs which are desirable in the mohair yarn and which will readily take a dye, but also 60 more or less of the so-called kemp hair or fibre which is relatively coarse and stiff, and which is white and will not take a dye.

If in making mohair yarn the kemp 65 fibres are left in the yarn it will, when dyed, present a streaky appearance due to the

presence of the white undyable kemp fibres. Consequently, it has heretofore been necessary to comb the fleece of the Angora goat until all the kemp fibre is removed before spinning the yarn therefrom. In combing out the kemp fibre many of the fine, soft fibres are lost and as a result the mohair 70 yarn is relatively expensive.

With my invention I find that it is possible to use a mohair yarn for the pile thread 75 which has more or less of the kemp fibre therein without in any way detracting from the appearance of the fabric.

When the pile fabric is woven with the light-colored or undyed warp threads, such 80 threads will be slightly visible on the pile face of the fabric especially at such places as the fabric may be doubled back on itself. The extent to which the light colored or white undyed warp threads show on the pile. 85 face of the fabric is not sufficient to give the face of the fabric a speckled or undesirable appearance but it gives the front of the fabric a sufficiently variegated appearance 90 to break up any streaky appearance which 95 might result from the presence of the kemp fibres in the pile threads. Wherever a kemp fibre appears in the pile face or pile ends it will tend to show because of the fact that it is stiffer and somewhat coarser than the 100 other fibres of the mohair yarn and because it retains its white appearance since it will not take a dye. The presence of these kemp 105 fibres would tend to give the pile surface of the fabric a more or less streaky appearance 110 but where the fabric is made with light-colored or undyed binder warp threads the light color of such warp threads shows through the pile face of the fabric to a sufficient extent to break up the streaky appearance due to presence of the kemp fibres. 115 In a fabric having the undyed warp threads as above described the portion of the warp threads which shows through on the 120 face of the fabric will be lighter in color 110 than the pile ends and this lighter color is what helps break up the streaky appearance due to the presence of the kemp fibres.

With my invention, therefore, it is possible to make an entirely satisfactory plush 125 by using for the pile threads a mohair yarn having more or less of the kemp fibres therein. Such a yarn is considerably less expensive than one from which all the kemp 130 fibres are removed and hence for this reason also my invention results in decreasing the cost of the manufacture of pile fabric.

Another advantage resulting from my invention is that the use of light-colored 135 warp threads facilitates the weaving of the fabric because the weaver can see the weaving operations much better and can watch his work with much less tiring effect on the eyes than when weaving on dark colored 140 warp threads. Furthermore, there is an 145

- added advantage when undyed warp threads are used because the undyed warp threads are considerably stronger than the dyed warp threads and an undyed warp will usually have very many less knots in it than a dyed warp. This is because the stronger undyed warp threads are much less liable to break in the warping and weaving processes than the weaker dyed warp threads.
- 10 The expression "undyed warp threads" as used above is not necessarily limited to warp threads which are made entirely of undyed fibres. Under some circumstances it may be desirable to use a warp thread 15 which is of a mixture of dyed and undyed fibres. Such a warp thread might result from spinning a mixture of undyed and dyed fibres or by twisting together a strand of undyed fibres and a strand of dyed fibres.
- 20 Hence the term "undyed warp threads" as used herein is intended to cover threads which are made either entirely or partially of undyed fibres.

It is the light color of the warp threads 25 which is effective in breaking up the streaky appearance caused by the presence of the kemp fibres in the pile threads and hence so far as this feature of the invention is concerned the desirable light or white color 30 for the warp threads may be secured in any suitable way.

The operations of scouring, dyeing or 35 finishing fabric after it comes from the loom are in no ways affected by the presence of the pyroxylin coating. In some fabrics, such for instance as those in which the pyroxylin coating is relied upon for binding the pile threads into the fabric or for giving strength to the fabric, it is highly desirable 40 that the coating should be applied just after the fabric comes from the loom and before it is subjected to the subsequent finishing operation because the presence of this coating will prevent injury to the fabric while 45 it is being finished. In other fabrics, where the pyroxylin coating is not required for giving strength to the fabric during the finishing operations such coating may be applied either before or after said finishing 50 operations or at any stage after the fabric leaves the loom.

As stated above I have, for convenience, used herein the term "pyroxylin" as descriptive of the flexible non-penetrating water- 55 and heat-resistant coating material but the invention is not necessarily limited to a pyroxylin material as any coating material having the desired characteristics would answer the purpose. Hence the term "pyroxylin" is used herein as indicating a material having the above characteristics rather than having certain chemical ingredients. The drawing shows in a conventional way 60 a pile fabric embodying the invention. The warp threads are indicated at 1, the filling

threads at 2, and the pile ends at 3, and the binding material at 4. It is to be understood however, that the drawing is not intended to illustrate a fabric structure except in a conventional way. The particular way of interlocking the warp threads, the filling threads and the pile ends vary with the character of the pile fabric and as my invention is applicable to pile fabrics in which the various threads comprising the fabric are interwoven in different ways, I have thought best to simply show the fabric conventionally in the drawing.

I claim:

1. A pile fabric having pile threads interlocked with interwoven filling threads and undyed warp threads, there being a deficiency of warp threads for binding the pile threads into the fabric, the back face of the fabric having a coating of colored pyroxylin applied thereto which by its adherence to the exposed portions of the pile threads and warp threads not only binds the pile threads into the warp threads but also colors the portions of the undyed warp threads that are exposed on the back of the fabric.

2. A pile fabric comprising pile threads of mohair yarn having kemp fibres therein, said pile threads being interlocked with interwoven filling threads and undyed warp threads, said undyed threads showing through the pile face of the fabric sufficiently to break up the streaky appearance caused by the presence of the kemp fibres in the pile threads.

3. The method of making a pile fabric which consists in interweaving pile threads, filling threads and undyed binder warp threads and then applying to the back of the fabric a coating of colored pyroxylin.

4. The method of making a pile fabric which consists in interweaving mohair pile threads having kemp fibres therein with filling threads and undyed warp threads, and then applying a coating of colored pyroxylin to the back of the fabric.

5. The method of making a pile fabric which consists in interweaving pile warp threads, filling threads and undyed warp threads, and in so doing employing a deficiency of warp threads for normally tying the pile threads into the fabric, and then applying to the back face of the fabric a coating of colored binding material which not only makes good the deficiency in the number of warp threads but also applies a colored coating to the portions of the undyed warp threads which are exposed on the back of the fabric.

6. A pile fabric having pile threads interlocked with interwoven filling threads and warp threads having undyed fibres therein, there being a deficiency of warp threads for binding the pile threads into the fabric, the back face of the fabric having a coating of

colored pyroxylin applied thereto which by its adherence to the exposed portion of the pile threads and warp threads not only makes good the deficiency in the warp threads but also colors the portions of the warp threads exposed on the back face of the fabric.

7. A pile fabric having pile threads interlocking with interwoven filling threads and warp threads, the latter being threads with undyed fibres therein, and there being a deficiency of warp threads for binding the pile threads into the fabric, the back face of the fabric having a coating of colored water-  
15 and heat-resistant, non-penetrative material which normally adheres to the portions of the thread exposed on said back face and thus makes good the deficiency in warp threads and which also applies a colored  
20 coating to the portions of the warp threads exposed on said back face.

8. A pile fabric having pile threads interlocked with interwoven filling threads and undyed warp threads, said undyed threads  
25 showing through the pile face of the fabric and the back face of the fabric having a coating of colored binding material applied thereto which by its adherence to the exposed portions of the pile threads and warp threads  
30 not only binds the pile threads into the warp threads but also colors the portion of the undyed warp threads that are exposed on the back of the fabric.

9. A pile fabric comprising pile threads of  
35 mohair yarn having kemp fibres therein, said pile threads being interwoven with filling threads and warp threads which are lighter in color than the pile threads, said warp threads showing through the pile face  
40 of the fabric sufficiently to break up the streaky appearance caused by the presence of the kemp fibres in the pile threads.

10. A pile fabric having pile threads interlocked with interwoven filling threads and warp threads which are lighter in color than the pile threads, said warp threads showing through the face of the fabric and the back face of the fabric having a coating of colored binding material applied thereto which by  
45 its adherence to the exposed portions of the pile threads and warp threads not only binds the pile threads into the warp threads, but also colors the portion of the warp threads that are exposed on the back of the fabric.

55 In testimony whereof, I have signed my name to this specification.

WILLIAM S. NUTTER.